

Patented Mar. 17, 1942

2,276,315

# UNITED STATES PATENT OFFICE

2,276,315

## TANNING

Joseph S. Kirk, Cleveland, Ohio, assignor to E. I.  
du Pont de Nemours & Company, Wilmington,  
Del., a corporation of Delaware

No Drawing. Application June 4, 1941,  
Serial No. 396,565

13 Claims.

(Cl. 149—5)

This invention relates to the production of leather and it is more particularly directed to compositions and processes for the tanning of skins with silicic acid sols containing a hydrogen bonding donor compound.

Silicic acid sols have been proposed as tanning agents but their use has been none to successful. It has been proposed to add various metal compounds such as aluminum or iron salts, but the modification has not led to satisfactory results. Tanning agents including silicic acid sols show so great an affinity for skin substance that over-tanning usually occurs. The leather produced is harsh, stiff, and of a generally unsatisfactory character. Changes occur in leather tanned with silicic acid sols according to the processes proposed in the art and the leather soon becomes even stiffer, sometimes to the point of brittleness.

It has further been proposed to modify so-called silica sol tanning agents by the inclusion of various organic compounds such as lactic acid and sulfite cellulose waste, but the addition of such modifying agents has not effected sufficient improvement in the tannages to make them satisfactory. The leather produced is still of poor character and has only a poor quality compared with standard vegetable and chrome tans which have found acceptance in the trade.

It is an object of this invention to provide novel tanning processes and compositions. It is a further object to provide tanning compositions and processes which produce a good quality of leather at relatively low cost. It is a further object of this invention to provide compositions and processes employing silicic acid sols in the tanning of skins to produce leather of good character. It is a still further object to provide processes and compositions which permit rapid, simple, and easily-controlled tanning of skins. It is a still further object of this invention to improve upon prior art processes employing silicic acid sols for the tanning of skins. It is a still further object of this invention to produce white leather. Still further objects will become apparent hereinafter.

The foregoing and other objects of this invention are attained by the use of a water-soluble hydrogen bonding agent with a silicic acid sol. By the inclusion of a hydrogen bonding donor compound in silicic acid tanning agents there are obtained tannages which are easily used and which are economical. Leather produced according to the preferred processes of this inven-

tion is of excellent character being opaque, soft, "full," and flexible.

The silicic acid sols used as tanning agents according to this invention are ordinarily produced by lowering the pH of a solution of a soluble silicate. When first formed the sols probably contain considerable amounts of silicic acid but silicic acid is probably present as such only for a relatively short time and then conversion to silica begins. Most silicic acid sols are, as is well-known, to an extent unstable and after a period of time varying from a few hours and upwards change over to a silica gel.

As has been the practice heretofore, silica sols should be used as tanning solutions before gelling occurs and before they become too astringent. It will generally be preferable to use these silicic acid sols shortly after they are made up even though sols modified with hydrogen bonding donor compounds according to this invention are of increased stability.

Silicic acid sols for use as tanning agents according to this invention may be prepared in various other ways already known to the art. It will ordinarily be desirable to start with a soluble silicate such as sodium or potassium silicate and reduce the pH of the silicate by adding it to an acidic material. Any acidic material may be used though as will be pointed out hereinafter certain acidic metal salts themselves have an effect in the resulting product. There may be used for reducing the pH of a silicate such acidic materials as sulfuric acid, sulfamic acid, hydrochloric acid, nitric acid, thionic acids, acetic acid, lactic acid, and other similar inorganic and organic acids. Acidulous salts may similarly be used and there may be employed for instance, sodium bisulfate, monosodium phosphate, acid tartrates, zinc chloride, titanium sulfate, aluminum sulfate, and chromium sulfate. The amount of acid or acidic material will ordinarily be such as to result in a pH of about 1.0 to 5.0.

It will ordinarily be desirable to reduce the pH of a silicic acid sol to about 1.5 to 3.5. Still more specifically as will be pointed out hereinafter, it will be preferred to reduce the pH to about 2.0 to 3.0. It will be understood that while any acidulous material may be used to increase the acidity of silicate solutions to produce silica sols, some acidulous materials do not themselves have a low enough pH to produce the final acidity desired. In this event such an acidulous material may be used in combination with a more acidulous material, and as will be evident mixtures

of two or more acidulous materials may be used as seems desirable.

There may be included in the silicic acid sols various metal compounds. If an acidulous metal compound is selected it may serve to supply a part or all of the acidity needed to produce the sol. There may be included in silicic acid sols according to this invention such metal cations as aluminum, chromium, iron, zinc, and titanium. These metals may be added in the form of any of their soluble compounds and there may be used, for instance, aluminum sulfate, aluminum formate, aluminum lactate, aluminum chloride, chromium sulfate, titanium sulfate, and iron sulfate.

The preferred tanning compositions according to the present invention are comprised of silicic acid sols containing a soluble aluminum compound. Aluminum is preferably introduced into a silicic acid sol in the form of aluminum sulfate, due consideration being given to the acidity of this compound so that the final pH will fall within the range desired. The amount of aluminum introduced should be such that the  $\text{Al}_2\text{O}_3:\text{SiO}_2$  ratio lies between the limits of 1:2 to 1:4 parts by weight. With much smaller ratios than 1:2 excessive puckering of the leather takes place and above about the 1:4 ratio the leather tends to become flat and tinney. The ratio of  $\text{Al}_2\text{O}_3:\text{SiO}_2$  can be obtained, as has been indicated above, by the use of various silicates and aluminum compounds with various acidulous materials as required.

The concentration of silicic acid sols may be selected as in prior processes with this sol. Sols made up for use may contain about four per cent  $\text{SiO}_2$  and two per cent  $\text{Al}_2\text{O}_3$  by weight. I have used 6 per cent  $\text{SiO}_2$  and 3 per cent  $\text{Al}_2\text{O}_3$ . Upon dilution to make a tanning bath it will seldom be found desirable to have an  $\text{SiO}_2$  content in excess of about two per cent.

According to the present invention silicic acid tanning agents are modified by the inclusion of a hydrogen bonding donor compound. Hydrogen bonding is a concept advanced in recent years to explain certain abnormalities in the chemical and physical behavior of mixtures of compounds one of which contains hydrogen attached to a strongly negative radical and the other an atom capable of donating a pair of electrons to form a directional or co-ordination bond. Since the bond is formed by the donation of an electron pair from one atom, the donor, to the other atom the bond is not of the type conceived as an ordinary valence bond but many of the properties of the mixture indicate that a type of chemical compound is formed. These mixtures, for instance, exhibit an abnormal vapor pressure lowering, that is abnormal deviation from Raoult's law. There is further observed abnormal heats of mixing and abnormal deviation in viscosity and freezing point lowering.

I have found that when silicic acid is mixed with an organic hydrogen bonding donor compound it exhibits characteristics unexplainable upon the basis of ordinary chemical reaction and unexpected from a consideration of the characteristics of the materials mixed. Apparently silicic acid has an acceptor hydrogen atom and forms some type of compound with a hydrogen bonding donor. Among the characteristics of these silicic acid-hydrogen bonding donor combinations is a decreased tendency to precipitate gelatin and an increase in the time required for the sol to be converted to the gel.

It will be understood that in advancing the theory of hydrogen bonding to explain the unexpected results of the present invention I do not intend to be limited or restricted by this theory.

6 The theory may or may not be correct and for purposes of the present invention it is of importance largely because whatever the reason, the type of compounds known to be organic hydrogen bonding donors profoundly modify silicic acid sols and gels.

It will be seen that these hydrogen bonding donor compounds are of the type of materials which might be designated as weak organic bases. According to this theory the materials involved

15 act as bases with silicic acid which is quite a strong acid. These bases are of such weakness that they will not raise the pH of a silicic acid solution above 7. According to this theory one

20 may therefore describe the agents added to silicic acid sols according to the present invention as water-soluble, organic bases which will not raise the pH of silicic acid above 7. It is again observed that while the terminology of either the "hydrogen bonding" theory or the "weak base" theory may advantageously be used in describing the present invention to those skilled in the art in commonly understood language applicant does not consider the adoption of either theory as bearing upon the invention save as it gives a convenient system of terminology.

30 While any hydrogen bonding donor compound (or weak base) may be used with silicic acid according to the present invention it will generally be found desirable to use any water-soluble hydrogen bonding donor compound selected from the group consisting of ethers, amides, alcohols, and ketones.

35 Silicic acid tanning agents prepared according to this invention are used in aqueous solution and 40 hydrogen bonding donor compounds used should accordingly be water-soluble at least to the slight extent required to permit formation of a co-ordination complex with silicic acid. Preferably, the donor compound should be water-soluble. 45 The structure of such materials as NN'-diphcnyl urea, diethyl ether, and N,N-dibutylstearamide might indicate that they would be satisfactory, but actually the compounds are too insoluble in water to serve as hydrogen bonding agents in 50 aqueous solution.

In addition to being water-soluble a hydrogen bonding donor should not contain groups which will react with silicic acid to give compounds of the conventional sort when such reaction would 55 interfere with hydrogen bonding. The donor preferably should not react with silicic acid to give a precipitate.

As has been indicated, the water-soluble, organic hydrogen bonding donor compounds used according to this invention are preferably selected from the group consisting of ethers, amides, alcohols, and ketones. It is preferred that the ethers have an oxygen or nitrogen atom in addition to that in the ether linkage and specifically it is desirable that the ether contain in addition to the ether group a second ether group, a hydroxy group, an amide group, or an ester group. Amides for use with silicic acid sols according to the present invention are preferably N-substituted. Alcohols for use as donors ought to contain more than two carbon atoms. Alcohols are among the weakest of the hydrogen bonding agents but may find value in some instances. Ketones are not quite as weak as alco-

hols and any water-soluble ketone may be used as above discussed.

Hydrogen bonding agents for use with silicic acid sols may be characterized by the description that they are non-alkaline, organic compounds containing at least one electro-negative atom selected from the group consisting of nitrogen and oxygen to which is attached no more than (X-1) hydrogen atoms where X is the minimum normal valency of the electro-negative atom, and to which hydrocarbon groups are attached by the other valences, there being in the donor compound a number of carbon atoms no less than two and at least twice as large as the number of hydrogen atoms attached to said electro-negative atom. This description of course omits ureas which are, however, specifically described and claimed in my co-pending application Serial Number 355,606, filed September 6, 1940.

As has been indicated above, ethers are among the preferred hydrogen bonding donor compounds for use with silicic acid sols according to the present invention. In addition to containing an ether group these donors may advantageously contain an additional ether group, a hydroxy group, an amide group, or an ester group. The presence of these groups appears very beneficial. A number of such groups may be present and there may be used, for instance, polyethers which contain hydroxyl groups and ester groups. As examples of ethers the following are listed:

Nonaneethylene glycol  
Dimethyl ether of tetraethylene glycol  
Dimethyl ether of diethylene glycol  
Hexaethylene glycol  
Butyl ether of diethylene glycol  
Ethyl ether of diethylene glycol acetate  
Methyl ether of diethylene glycol acetate  
Tetraethylene glycol  
Monoethyl ether of diethylene glycol  
Triethylene glycol  
Monoethyl ether of ethylene glycol  
Monomethyl ether of ethylene glycol  
Diethylene glycol  
N,N'-bis(beta-methoxyethyl) adipamide  
N,N'-bis(methoxymethyl) urea  
Polyethylene glycol adipate  
Diethyl ether of diethylene glycol  
Dioxane  
Dioxolane  
Diethyl ether of ethylene glycol  
Dimethyl ether of ethylene glycol  
Triethylene glycol dipropionate  
Glycerol formal  
Ethylene glycol acetal  
Sorbitol triacetal  
N,N-dimethylmethoxyacetamide  
N-acetylmorpholine  
N,N'-adipylmorpholine  
Dimorpholide urea  
Polyethylene oxide  
Monomethyl ether of ethylene glycol-ethylene oxide reaction product  
Ethylene glycol-ethylene oxide reaction product  
Glycerol-ethylene oxide reaction product  
Ethanolformamide-ethylene oxide reaction product

Amides are among the preferred hydrogen bonding donors for use with silicic acid sols according to this invention. Whereas oxygen is the donor atom in ethers the nitrogen of amides probably acts as the donor atom. Among the most effective compounds of this group are the N-substituted amides and the di-substituted

compounds are preferred. It will be seen that some of the compounds in the above list of ethers are amides as well and could have been shown below as illustrative of the use of amides. The use of amides specifically in tanning is covered in my aforementioned application Serial Number 355,606, filed September 6, 1940.

Examples of amides are listed below, ureas and other amides being listed separately:

#### Ureas

Tetramethylurea  
Tetraethylurea  
Urea  
Thiourea  
N,N'-diethyl-N,N'-diethanolurea

#### Amides

N,N,N',N'-tetramethyladipamide  
N,N-dimethylacetamide  
N,N,N',N'-tetramethylsuccinamide  
N,N,N',N'-tetraethylsuccinamide  
N,N-diethylacetamide  
N,N',N'-tetraethyloxamide  
N,N'-diethylformamide  
N,N-diethylpropionamide  
N,N-dimethylformamide  
N,N,N',N'-tetraethyloxamide  
N,N-diethylglycolamide  
N-ethyl-N-ethanolformamide  
N-ethyl-N-ethanolglycolamide  
N-(2,3-dihydroxypropyl) methoxyacetamide  
N-butyl-N-beta-hydroxyethylactamide  
N-ethanolethanesulfonamide  
N-isobutylacetamide  
N,N'-diethanoloxamide  
N,N'-diethanolsuccinamide  
N-formylhexamethylenimine  
Diethylcyanamide  
Acetamide  
Succinamide  
Formamide

Examples of ketones may be given as follows:

#### Ketones

45 Acetonylacetone  
Acetone  
Formacetoethyl  
Methyl acetoacetate  
50 Diacetone alcohol

Examples of alcohols may be given as follows:

#### Alcohols

Diacetone alcohol  
65 2-methyl-2,4-pentanediol  
Isopropanol  
Pinacol  
Hexamethylene glycol  
Pentaglycol  
60 Tert-butyl alcohol  
Tetrahydroxy octane  
1,1,1-trimethylolethane  
Propanediol

Silicic acid sols for use as tanning agents according to the present invention are preferably formed in the presence of a hydrogen bonding donor compound, but if desired the donor may be added to a freshly-prepared sol. The amount of hydrogen bonder to use in a particular case varies considerably with the results desired and with the particular silicic acid sol and the particular tanning procedure chosen. The amount of donor should of course not be so great as to slow the tanning down unduly and yet it should

be sufficient to prevent too rapid a tanning. The precise amount of a particular agent to use in a particular tanning bath can best be determined by a few simple trials. In general, it may be indicated that there should be used an amount of donor equivalent to from about 0.1 per cent to 10 per cent of the weight of the tanning solution.

The silicic acid sol tanning agents of this invention may be used for the treatment of any type of skin adapted to be converted into leather or fur. It is to be observed that the term "skin" is used generically to include heavy skins such as cowhide, lighter skins such as goatskin and calfskin, and also skins of fur-bearing animals. It will naturally be necessary to adapt the processes to the type of skin to be treated. For instance, goatskin may be more rapidly tanned than calfskin, but those skilled in the art are well aware of such factors and may readily adapt the compositions of this invention to the specific needs of particular specialized problems.

Skins to be tanned according to the processes of this invention may be prepared in any of the manners customary in the art. They may suitably be unhairied, limed, delimed, and bated and pickled. The skins may if desired be de-pickled. They may also be given a salt liquor treatment to soften them and to put them in a more uniform condition as is the practice in prior art tanning processes.

While skins prepared in any manner may be treated according to the processes of this invention, the pH of the skins is important. As will be observed below, the tanning is effected at certain conditions of acidity and the skins may tend to change these conditions. The tanning solution may suitably be controlled to compensate for variance of the pH of the skins from that of the tanning solution. It may sometimes be found advantageous to adapt the processes for preparing the skins so that a skin prepared for tanning is approximately at the pH of the tanning solution.

Too rapid reaction of the tanning agent with the skins in the first stages of the process should be avoided in order to prevent surface hardening of the skin. The amount of hydrogen bonding donor used should, as indicated above, be such as to assist in preventing too rapid a tanning and the initial pH of the solution should not be too high. The initial pH of the solution will ordinarily be from about 1.5 to 3.0. More specifically, it will be found preferable to use a pH of about 2.5. If the initial pH is much above 3.5 the tanning will proceed too rapidly in the initial stages though it will be understood that the pH to be selected in any particular instance will depend upon the specific conditions of the tannage. If too low a pH is used combination of silica with the skin is too slow and, additionally, excessive acidity may deleteriously affect the skin.

After satisfactory penetration has been obtained the pH of the solution is raised by the addition of any suitable alkali. Raising the pH accelerates the tanning action. The pH should at this point be raised to about 3.5 to 4.5. Sodium carbonate or other alkali metal or ammonium hydroxides or carbonates or organic bases such as ethanolamines may be used to raise the pH.

The considerations as to the type of apparatus to use, the time to be allowed for tanning, the temperatures of tanning, and the amounts of tanning agent are substantially those known to the art in connection with prior art tanning

processes. The time allowed for tanning must be sufficient to permit complete penetration of the tanning agent, and the pH should not be raised too rapidly or there may be puckering and apparent over-tannage of the grain surface. The tanning can best be effected at room temperature, say 20° to 30° C. The exact amount of the tanning solution to use can best be determined by a few simple tests under the specific conditions of the process selected and with the specific skin to be treated. In general, enough of the tanning agent must be used to effect the tanning desired but unduly large amounts should not be used as they will not be taken up by the leather in a reasonable period of time and they may cause over-tannage.

The leather obtained according to the preferred processes of this invention using a silicic acid sol with a soluble aluminum compound is white, but it may if desired be treated with white pigment or may be colored during or after the tanning processes by inclusion of any of the common leather dyes and pigments. Leather produced by any of the processes of this invention may similarly be colored and dyed in accordance with the practices known in the art.

Silicic acid sol tanning agents, including a hydrogen bonding donor according to the present invention may if desired be used with other tanning agents or tanning assistants heretofore known to the art. They may, for instance, be used in conjunction with vegetable tanning materials such as quebracho extract, with chrome tans, or with synthetic tanning agents such as those containing sulfonic acid groups. The silica sols may be used to begin tanning and other tanning agents used to finish off the leather, or alternatively, the other tans may be used to begin the tanning and the silicic acid sols used for finishing. When other tanning agents are used simultaneously with the silicic acid sols due consideration must of course be given to the acidity of the resulting solution so that it will fall within the ranges heretofore mentioned.

As has been suggested in the foregoing, the tanning solutions may contain any of the various additions suggested by the art as beneficial in silicic acid sols. Suitable dispersing or stabilizing agents may be used as desired and in general the practices in the art with respect to silica sols may advantageously be employed in specific instances.

The tanning agents of this invention may be offered to the trade as sols containing a hydrogen bonding donor compound and additionally containing metals and other assistants as desired. If it is likely that the tanning agents will not be used for quite awhile it may be found preferable to sell two components, one, for instance, containing sodium silicate and any suitably modifying agents which do not lower the pH to a point so low that a sol is formed, and a second component containing a hydrogen bonding donor compound and an acidic material in such amount that when the two components are mixed a sol of substantially the character desired will be obtained. Naturally the second component like the first may include various modifying agents and tanning assistants and if a soluble metal compound is to be used it will ordinarily be found preferable to include it in the second component.

Leather produced according to the processes of this invention may be subjected to any of the various kinds of finishing treatments customarily

used. The leather, if desired, may be suitably filled or given any of the numerous surface treatments customary in the art.

My invention will be better understood by reference to the following illustrative examples:

EXAMPLE 1

A tanning solution was prepared according to the present invention by making up the A and B solutions as tabulated and adding solution B to solution A with agitation. The tanning solution was clear and had a pH value of 2.4. In the following parts are given as parts by weight:

*Solution A*

|                                                                          | Parts |
|--------------------------------------------------------------------------|-------|
| 20% sulfuric acid                                                        | 7.12  |
| Water                                                                    | 21.00 |
| Methyl ethyl ketone                                                      | 0.65  |
| Aluminum sulfate $\text{Al}_2(\text{SO}_4)_3 \cdot 18\text{H}_2\text{O}$ | 9.80  |

*Solution B*

|                                                                        | Parts |
|------------------------------------------------------------------------|-------|
| 42.5° Bé. sodium silicate ( $\text{Na}_2\text{O}:\text{SiO}_2$ ) ratio |       |
| 1:3.25                                                                 | 10.12 |
| Water                                                                  | 22.00 |

In a tanning drum there was placed 50 parts (drained pickled weight) of goatskins which had been unhairied, delimed, and pickled in customary manner. The skins were agitated for ten minutes with 50 parts of a 10 per cent solution of sodium chloride and then the tanning solution prepared as above was added. The skins were agitated and were neutralized to pH 4.3 during the course of one hour and forty minutes by repeated additions of a 10 per cent solution of sodium bicarbonate. The skins were removed from the drum and piled down over night.

The skins were returned to the drum containing the tanning solution and neutralization continued to pH 5.8. The skins were then washed and fatigued and after drying, stacking, and tacking the resulting leather was smooth, white, full, and supple.

EXAMPLE 2

A tanning procedure was used as shown in Example 1 but using instead of the sol of Example 1 the following:

*Solution A*

|                   | Parts |
|-------------------|-------|
| Sulfuric acid     | 7.12  |
| Water             | 21.00 |
| Diacetone alcohol | 1.00  |

|                                                                  | Parts |
|------------------------------------------------------------------|-------|
| 42.5° Bé. sodium silicate ( $\text{Na}_2\text{O}:\text{SiO}_2$ ) | 10.12 |
| Water                                                            | 22.00 |

Leather of good quality was produced.

EXAMPLE 3

A tanning procedure was followed as in Example 1 using a tanning solution made up with the following:

*Solution A*

|                        | Parts |
|------------------------|-------|
| 20% sulfuric acid      | 7.12  |
| Water                  | 21.00 |
| Tertiary butyl alcohol | 1.00  |

75

*Solution B*

|                                                                        | Parts |
|------------------------------------------------------------------------|-------|
| 42.5° Bé. sodium silicate ( $\text{Na}_2\text{O}:\text{SiO}_2$ ) ratio |       |
| 1:3.25                                                                 | 10.12 |

5 Water

22.00

Leather of good quality was produced.

EXAMPLE 4

A tanning procedure was followed as in Example 1 using a tanning solution made up with the following:

*Solution A*

|                     | Parts |
|---------------------|-------|
| 20% sulfuric acid   | 7.12  |
| 18 Water            | 21.00 |
| Nonaethylene glycol | 0.40  |

Aluminum sulfate

9.80

*Solution B*

|                                                                        | Parts |
|------------------------------------------------------------------------|-------|
| 42.5° Bé. sodium silicate ( $\text{Na}_2\text{O}:\text{SiO}_2$ ) ratio |       |
| 1:3.25                                                                 | 10.12 |

Water

22.00

Leather of good quality was produced.

EXAMPLE 5

A tanning procedure was followed as in Example 1 using a tanning solution made up with the following:

30

*Solution A*

|                        | Parts |
|------------------------|-------|
| 20% sulfuric acid      | 7.12  |
| Water                  | 21.00 |
| Butyl carbitol acetate | 0.75  |

35

Aluminum sulfate

9.80

*Solution B*

|                                                                        | Parts |
|------------------------------------------------------------------------|-------|
| 42.5° Bé. sodium silicate ( $\text{Na}_2\text{O}:\text{SiO}_2$ ) ratio |       |
| 1:3.25                                                                 | 10.12 |

40

Water

22.00

The leather produced was of good character.

While I have shown certain illustrative tanning compositions and processes it will be understood that without departing from the spirit of this invention one skilled in the art may readily use various water-soluble hydrogen bonding donor compounds with silicic acid sols in a wide variety of ways.

50 This application is a continuation-in-part of application Serial Number 355,605, filed September 6, 1940.

I claim:

53 1. A tanning composition comprising a silicic acid sol and a water-soluble, organic hydrogen bonding donor compound.

2. A tanning composition comprising a silicic acid sol, a water-soluble hydrogen bonding donor compound, and a soluble aluminum compound.

60 3. A tanning composition comprising a silicic acid sol, a water-soluble ether, and aluminum sulfate.

4. In a tanning process, the step comprising subjecting a skin to a tanning solution comprising a silicic acid sol and a water-soluble, organic hydrogen bonding donor compound.

65 5. In a tanning process, the step comprising subjecting a skin to a tanning solution comprising a silicic acid sol and a water-soluble ether.

6. In a tanning process, the step comprising subjecting a skin to a tanning solution comprising a silicic acid sol and a water-soluble ether which has an oxygen or nitrogen atom in addition to that in the ether linkage.

7. In a tanning process, the step comprising

subjecting a skin to a tanning solution comprising a silicic acid sol, a water-soluble hydrogen bonding donor compound, and a soluble aluminum compound.

8. In a tanning process, the step comprising subjecting a skin to a tanning solution comprising a silicic acid sol, a water-soluble ether, and aluminum sulfate.

9. In a tanning process, the step comprising subjecting a skin to a tanning solution comprising a silicic acid sol and a water-soluble, organic hydrogen bonding donor compound.

10. A tanning composition comprising a silicic acid sol and a water-soluble alcohol.

11. A tanning composition comprising a silicic acid sol and a water-soluble ketone.

12. In a tanning process, the step comprising subjecting a skin to a tanning solution comprising a silicic acid sol and a water-soluble alcohol.

13. In a tanning process, the step comprising subjecting a skin to a tanning solution comprising a silicic acid sol and a water-soluble ketone.

JOSEPH S. KIRK.